

## UNITED STATES PATENT OFFICE.

JOSEPH T. TERRY, OF ALHAMBRA, CALIFORNIA, ASSIGNOR TO CORDELIA E. TERRY,  
OF ALHAMBRA, CALIFORNIA.

## CONCENTRATION OF OXIDIZED ORES.

No Drawing.

Application filed November 23, 1925. Serial No. 71,019.

This invention relates to a process of treating ores and other metal bearing materials.

It is an object of this invention to provide a process which is simple, efficient and of sufficient economy to render concentration practicable.

My invention is based on my discovery that chromium salts of metallic elements substantially insoluble in the solutions employed are susceptible to flotation concentration and also that lead, zinc, silver, bismuth and mercury minerals are converted to substantially insoluble chromium derivatives by treatment with solutions of alkali metal chromates or alkali earth metal chromates alone or in conjunction with other reagents.

My process contemplates briefly the subjecting of the metalliferous material to the action of the water soluble chromates, such as sodium chromate or bi-chromate in neutral solutions or in conjunction with a neutral salt such as sodium chloride or an alkali such as caustic soda or alkaline compounds such as sodium carbonate, sodium silicate, aqua-ammonia or an acid such as sulphuric, hydrochloric or acetic acid, to convert the metal or metals at least in part to chromium compounds substantially insoluble in the solution employed. Only a partial conversion or superficial surface filming of the metalliferous particles is necessary for the success of my process. The part thus treated may then be subjected to any preferred method of froth flotation for the concentration and recovery of a concentrate containing chromium and other metal or metals associated therewith.

It is another object of my invention to treat ores containing two or more metals in such a manner as to first recover one of them by any suitable or preferred method, and then to recover the other metal or metals by the use of my treatment with chromates, or first with chromate to remove one of the metals and then to remove the other metal or metals in any suitable or preferred method, and in this manner, effect a separation as well as a concentration of metal bearing ores.

With the above and other objects in view, which will appear as the description proceeds, my invention consists in the steps of the process hereinafter described.

Assuming that an ore containing lead and

zinc both in the form of carbonates is to be treated, the ore is first ground to 65 mesh screen or finer, water is added to the ground ore and the mixture is rendered alkaline by the addition of any suitable base such as sodium hydroxide or salt having an alkaline reaction such as sodium carbonate, using approximately 2.5 grams of sodium hydroxide to 1 liter of water. To the mixture is now added sodium chromate  $Na_2CrO_4$ . The quantity of the latter will vary, depending upon the richness of the ore, but 1 gram to a liter is ordinarily sufficient. The proportion of the ore to the water is one part to four, the reaction takes place promptly, the sodium chromate combining with the lead and zinc in the ore, forming a corresponding chromate in accordance with the following chemical equation:



It will be understood that a mere filming action is necessary in this process. At ordinary temperature the reaction is complete in about one-half hour, but heating the mixture facilitates the reaction, for instance, heating to 180° F. will complete the reaction in about five minutes. The mixture is now conveyed to a froth flotation tank of any suitable or preferred construction, and subjected to a froth flotation agent such as ortho-tolidine. This flotation reagent will float the lead chromate only, leaving the zinc chromate unaffected. The remaining pulp is now treated with a froth flotation agent consisting of oleic acid and distillate, which will float the zinc chromate.

The liquid containing considerable quantities of unused sodium chromate is now decanted from the pulp, restandardized to make up the deficiency in sodium chromate and sodium hydrate and used in the treatment of another batch of ore.

As a modification of the above process in the treatment of an ore containing lead and zinc, whether in the form of carbonates or any other salt or oxide, the ground pulp is acidulated with sulphuric acid, using 2½ c. c. of sulphuric acid to the liter of water and using 2 grams of sodium chromate to the liter. In this acid solution the sodium chromate will react with the lead only, forming lead chromate and leaving the zinc unaffected. The mixture is then treated in the

flotation tank with a flotation agent such as oleic acid and carbon bi-sulphide or cresylic acid and distillate. After the removal of the lead chromate by flotation the pulp containing the zinc is rendered alkaline by the addition of sodium carbonate or sodium hydroxide when the sodium chromate will attack the zinc and form zinc chromate, which may then be floated by mixture of 10 oleic acid and distillate.

As a third modification of the treatment of the lead and zinc ore just referred to, the ground ore may first be treated with sulphuric acid sufficient in quantity to combine with all the zinc in the ore to form 15 zinc sulphate. The lead will form insoluble lead sulphate. The zinc sulphate in solution is decanted and the pulp containing now the lead alone is treated with sodium chromate to film the same with lead chromate, which may then be removed in the froth flotation tank by flotation agents such as oleic acid and carbon bi-sulphide or cresylic acid and distillate.

If the lead and zinc ore should contain silver, the latter combined with the lead, then the silver will be recovered together with the lead chromate, as described in the preceding processes. However, if the silver 30 is in the form of silver carbonate and not combined with the lead, then it will form silver chromate and be recovered together with the lead chromate.

Ores containing bismuth or mercury may 35 be treated in the same manner with sodium chromate in alkaline solutions, forming the corresponding bismuth chromate and mercury chromate are recovered by flotation.

My chromate filming process is applicable, 40 as mentioned before, to all ores other than sulphides. Sulphides are not included because they are floatable as such, and therefore require no treatment. However, I have found that a more effective extraction of 45 the metal content of some ores is obtained by treating the ores in an acid or alkaline solution with a chromate solution to form the corresponding metal chromate at least in part, and then by treating the mixture 50 with an agent such as sodium sulphide or hydrogen sulphide to form the corresponding metal sulphides. As well known, the metal sulphides are exceedingly floatable by well known froth flotation methods and 55 with some ores it may be economical because of the more effective recovery of the metal contents to use this modification of the process as explained, to-wit, first forming the metal chromate at least in part, and then the corresponding metal sulphide, which is 60 then recovered by froth flotation.

Another modification is to use sodium chromate in ammonical solutions in the treatment of zinc minerals other than sulphides. The ammonia of the solution ap-

pears to attack the zinc so that the latter is instantly filmed with the zinc chromate and may then be recovered by froth flotation with oleic acid and distillate. The use of ammonical solutions is also advantageous in 70 the treatment of lead minerals other than sulphides, but it is especially useful for zinc minerals.

In a similar manner ores other than sulphides containing bismuth, silver and mercury may be treated with chromate solutions to form a chromium derivative at least in part, so as to render the metal values floatable by well known froth flotation processes.

Any soluble chromate may be used, but 80 naturally sodium bi-chromate will be employed because of its low cost. It is of course understood that a base such as sodium hydroxide added to a bi-chromate solution converts it into the normal chromate.

Another modification of my process relates to the treatment of lead sulphide (galena) associated with lead carbonate and iron sulphides (pyrites). The ground ore pulp is first treated in the flotation tank with a suitable reagent such as a mixture of pine oil and carbon bi-sulphide, which will float the lead sulphide and leave the lead carbonate and iron pyrites unaffected. After the removal of the concentrate of lead sulphide 95 the ore pulp is rendered alkaline and sodium chromate is added, thereby forming lead chromate, at least in part, the iron pyrites remaining unaffected and the pulp is then submitted to froth flotation by the same or 100 other suitable reagents to recover the lead carbonate.

Methods have been known before in which ores containing lead minerals were treated to form a superficial film of lead chromate 105 and treating the same with an organic substance to oxidize the latter and precipitate the oxidation products on the particles of the lead minerals. My process differs therefrom in subjecting the finely ground ore 110 pulp, which has been treated with a chromate solution, at once without any oxidation process to a froth flotation.

Various changes in the steps of the process may be made by those skilled in the art 115 without departing from the spirit of my invention, as claimed.

I claim:

1. A process of treating ores other than sulphides, and containing lead, zinc, silver, 120 mercury and bismuth, either singly or in combination, comprising subjecting the finely ground ore pulp to a chromate solution to form the corresponding metal chromium derivative at least in part and directly 125 treating the ore pulp by a froth flotation process to concentrate the metal affected by the chromium treatment.

2. A process of treating ores other than sulphides, and containing lead, zinc, silver, 130

- mercury and bismuth, either singly or in combination, comprising subjecting the finely ground ore pulp to a chromate solution to form the corresponding metal chromium derivative at least in part and directly treating the ore pulp with a selective froth flotation agent to separately concentrate and recover the metals affected by the chromium treatment.
- 10 3. A process of treating ores other than sulphides, and containing lead, zinc, silver, mercury and bismuth either singly or in combination, comprising subjecting the finely ground ore pulp to an alkali metal chromate solution to form the corresponding metal chromate at least in part, and directly treating the ore pulp by a froth flotation process to concentrate the metal or metals affected by the alkali metal chromate treatment.
- 15 4. A process of treating ores other than sulphides and containing lead, zinc, silver, mercury and bismuth either singly or in combination, comprising subjecting the finely ground ore pulp to a chromate solution
- acid in reaction, thereby forming the corresponding metal chromium derivative at least in part of the metals capable of reacting with the chromate solution in an acid medium, treating the ore pulp by a flotation process to concentrate and remove the metal chromate derivative, rendering the ore pulp alkaline in reaction thereby forming metal chromium derivative of a metal capable of reacting with the chromate solution in an alkaline medium and directly treating the pulp by a froth flotation process to concentrate the metal chromium derivative thus formed.
- 20 5. A process of treating ores other than sulphides containing lead and zinc comprising treating the ore pulp with a chromate solution to form lead chromate at least in part and directly treating the pulp by a froth flotation process to concentrate and remove the lead chromate derivative.

In testimony whereof I have signed my name to this specification.

JOSEPH T. TERRY.